

A. G. JONES.

ORE REDUCING FURNACE.

APPLICATION FILED MAR. 26, 1914. RENEWED JAN. 20, 1916.

1,174,728.

Patented Mar. 7, 1916.

2 SHEETS—SHEET 1.



Witnesses:

*John Taylor*

*Irvin C. Bourman*

Inventor:

*Albert G. Jones*

*Boggy Creek, Lee, Christopher Miles,  
Al. 1115.*

A. G. JONES.

ORE REDUCING FURNACE.

APPLICATION FILED MAR. 26, 1914. RENEWED JAN. 20, 1916.

1,174,728.

Patented Mar. 7, 1916.

2 SHEETS—SHEET 2.



Witnesses:

E. G. Gaylord,  
T. W. Burnam.

Inventor:

Albert G. Jones,  
By D. Grumforth, Sec., Chittenden, Vt.,  
Attest.

# UNITED STATES PATENT OFFICE.

ALBERT G. JONES, OF IRON MOUNTAIN, MICHIGAN, ASSIGNOR TO NEW METALS-  
PROCESS COMPANY, OF CHICAGO, ILLINOIS, A CORPORATION OF ILLINOIS.

## ORE-REDUCING FURNACE.

1,174,728.

Specification of Letters Patent.

Patented Mar. 7, 1916.

Application filed March 26, 1914, Serial No. 827,357. Renewed January 20, 1916. Serial No. 73,177.

*To all whom it may concern:*

Be it known that I, ALBERT G. JONES, a citizen of the United States, residing at Iron Mountain, in the county of Dickinson 5 and State of Michigan, have invented a new and useful Ore-Reducing Furnace, of which the following is a specification.

This invention pertains particularly to furnaces adapted to the purpose of reducing metal oxides and carbonates to enable 10 the metal to be separated.

The primary object is to provide a furnace which is well adapted to metallize ores at a very low cost and produce the metals in 15 practically pure form.

The invention is illustrated in its preferred embodiment in the accompanying drawings, in which—

Figure 1 represents a broken elevational 20 view of a furnace embodying the invention; Fig. 2, an enlarged vertical sectional view of the same; and Fig. 3, a broken sectional view illustrating a slight modification.

In the embodiment illustrated, the invention 25 comprises a de-oxidizing chamber A in which the ore is reduced to a metallic state; a pre-heating device B wherein the de-oxidizing gases produced in the furnace are consumed and utilized in pre-heating 30 the ore and solid fuel as they pass to the furnace; and a chimney or stack C through which the products of combustion are discharged from the pre-heater B. The ore and fuel may be fed to the pre-heater B 35 from a hopper 1 having an inclined chute 2 which extends through the chimney and serves to discharge the materials into the upper end of the pre-heater.

The pre-heater preferably comprises a 40 cylinder mounted on rollers 3 and adapted to be slowly rotated by any suitable means (not shown). In the case of a furnace having a capacity of approximately 100 tons per day, such as would be afforded by a de- 45 oxidizing chamber having a diameter of approximately 20 feet and otherwise properly proportioned, it would be desirable to employ a pre-heating tube of approximately 8 feet in diameter and 120 feet in length. 50 The pre-heating tube B should be provided with suitable refractory walls to withstand a heat of at least 2000° F. The pre-heated ore and fuel are discharged through an elbow or hood 4 into a hopper 5 fitted with

a slide or closure 6 which may be withdrawn or opened at suitable intervals to permit the materials to drop into the furnace.

The chamber A is preferably of circular form and has the base-portion 5 provided 60 with a downwardly-tapering inner wall 5<sup>a</sup>, and has the semi-spherical upper wall 5<sup>b</sup>. At the junction of the upper and lower portions of the furnace is an annular bustle-chamber or bustle-pipe 7 into which the 65 gases pass through openings 7<sup>a</sup>. Communicating with the bustle-pipe 7 is an outlet flue 8 which communicates with the lower end of the pre-heater B, the flue 8 preferably extending through the elbow 4. The 70 lower portion of the chamber A should not be contracted sufficiently to cause choking, however.

Air is admitted to the upper portion of the chamber A through a twyer or tuyers 9 75 fitted with any suitable air-regulating valve 10. The tuyers 9 should be adapted to admit sufficient air to provide a de-oxidizing gas, but the air admission should be so controlled as to prevent complete combustion 80 within the furnace. In a furnace of the size indicated above, it is desirable to provide a plurality of tuyers. For illustration, one may use eight tuyers, each having a diameter of approximately twenty four 85 inches. The air preferably passes through the tuyers 9 by natural draft, but pressure may be employed if desired. The air may also be pre-heated if desired.

Through the upper inclined portion of the 90 flue 8 extends a twyer 11 fitted with an air-admission valve 12. The twyer 11 should be of sufficient capacity to admit enough air to the pre-heater B to complete the combustion of the inflammable gases which pass to 95 the pre-heating chamber through the flue 8. It is desirable to burn the combustible gases and utilize the heat therefrom for pre-heating, but a neutral or non-oxidizing medium should be maintained in the pre-heater. In 100 other words, the best results are obtained by supplying to the pre-heater air sufficient to burn the gases, but with no free oxygen present to attack the solid fuel.

The neck-portion of the furnace may be 105 provided with pipes 13 through which water may be circulated for cooling purposes. The upper portion of the furnace may be

fitted with removable plugs 14 received by poker-openings 15. In the base-portion of the furnace are provided discharge-chambers 16; and a discharge-slide 17, which may 5 be hydraulically actuated, is also provided. A cone 18 may serve to spread the burden; or any suitable means may be employed to insure proper drawing of the air through the burden.

10 The stack C should be of ample dimensions to give the desired draft, say, of a diameter of 8 feet and a height of 150 feet. The proportions for the stack and pre-heater which have been given are ample— 15 in fact larger than are necessary.

In the operation of the improved furnace, the ore and the bulk of the solid fuel (in distilled form) are fed through the hopper 1 to the slowly-revolving pre-heater B down 20 which the material gravitates and fills the furnace, the slide 6 being open. The upper portion of the mixed ore and fuel in the furnace assumes a position somewhat as indicated by the dotted lines 19. The slide 6 25 is then closed and the furnace fired at the base, which can be done by withdrawing the slide 17. The products of combustion pass up through the flue 8 and are discharged into the pre-heater. Sufficient air 30 is admitted through the twyers 9 to provide a de-oxidizing flame. Sufficient air is admitted through the twyer 11 to complete the combustion of the de-oxidizing gas which passes to the pre-heater through the flue 8.

35 In this manner the temperature in the lower portion of the tube B is raised to at least 2000° F. The temperature in the tube B gradually decreases as the stack is approached, and at the upper end of the tube 40 the temperature need not exceed approximately 500° F.

It is preferred to feed a mixture of ore and either coke or charcoal to the furnace through the pre-heater B in accordance with 45 the process described in the application of Albert G. Jones, No. 827,358, filed of even date herewith, using such an excess of the coke or charcoal in lump or block form as will serve to hold portions or lump-groups 50 of the ore separated or practically isolated from each other; and it is preferred to charge directly into the upper portion of the furnace, as through a door 20, a relatively small proportion of fresh carbonaceous fuel 55 adapted to supply hydrocarbons and hydrogen gas, as for instance, wood or coal.

In charging the furnace in the first instance through the pre-heater B, one may use either wood or coal, preferably in block 60 or lump form, mixed with the ore; and when the furnace is fired, coke or charcoal will be produced, which will be discharged with the metallized ore. Thereafter, the coke or charcoal may be separated from the 65 metallized ore and re-charged with fresh ore

into the pre-heater, and a relatively small amount of fresh coal or wood may be charged into the furnace from time to time through the charging-door 20.

In treating an ore composed mainly of iron oxid, a suitable mixture of coke and ore is afforded by using approximately 400 pounds of coke to 250 pounds of ore, supplemented by 100 pounds of coal introduced through the charging-door 20. The coke 75 is used over and over again until it is finally consumed, the fresh coal introduced through the door 20 serving continuously to replenish the supply of coke.

It is desirable not only to de-oxidize the 80 metal oxids, but also to "set" or "fix" the metals, so that reoxidation will not occur. This is accomplished by metallizing the ore and globing or globularizing the metal by producing in the furnace A a considerable 85 excess of heat over that required for de-oxidizing purposes, so that the metal particles which are grouped close to each other will fuse and form themselves into globular shapes, but without producing a molten 90 bath. The materials are discharged in solid form, but in separate lumps or pieces, at the bottom of the furnace.

Copper oxids and copper carbonates are amenable to the same treatment but require 95 somewhat less fuel, and the treatment may be carried on at a somewhat lower temperature. In operating the furnace on ores of the character above referred to, the temperature in the upper portion of the furnace 100 should be in excess of 2000° F. and preferably ranging as high as 3000° F. or higher. The temperature in the vicinity of the outlets 7<sup>a</sup> would be lower, but preferably should not fall much below 2000° F. It has been 105 found that when a sufficiently intense heat is maintained the carbon dioxide which is formed in the vicinity of the twyers 9 will give up a portion of its oxygen to the carbon, forming carbon mon-oxid, which, in 110 turn, robs the metal oxids of their oxygen. Under these conditions, there is a rapid interchange of oxygen, and the de-oxidizing of the metal oxids is rapidly effected. Such portions of the metals as become globed in 115 masses are readily separated from the fuel when the fuel is discharged from the furnace. On the other hand, myriads of tiny globules of metal may adhere to the coke and be re-charged therewith into the pre-heater, 120 and during a second journey through the furnace, these small metal globules carried by the coke coalesce with other metal globules, forming globules of tangible size which are readily recoverable.

In the case of zinc and lead, vaporization takes place at a temperature of approximately 2200° F., and a condenser is necessary to effect recovery. In dealing with lead and zinc oxids and carbonates, the furnace may 130

be operated at a somewhat lower temperature than is ordinarily desirable when dealing with iron and copper ores.

It may be added that owing to the fact 5 that the ore and fuel-pile in the furnace is of relatively small height and wide base, it is possible to operate the furnace by natural draft, thus effecting a very great economy; and the improved furnace may be so operated 10 as to produce practically perfect combustion before the gases are discharged from the pre-heater B into the stack. It will be understood, of course, that the hydrogen and hydro-carbons distilled from such fresh fuel 15 as is introduced through the door 20 will aid in the de-oxidizing process.

While it is unnecessary to use an air-blast in connection with the improved furnace, it is nevertheless possible to use the air-blast; 20 and where so used, comparatively small power would be required, owing to the low column of ore through which the gases must of necessity pass. In Fig. 3 is shown a modification in which the hopper 5 is replaced 25 by a charging-neck 5<sup>a</sup> equipped with bells 5<sup>b</sup> of known form, beneath which is a twyer 9<sup>a</sup> through which air is supplied from a fan 9<sup>b</sup>. Such an arrangement may be used, if desired, but natural draft will suffice. The 30 flue 8<sup>a</sup> corresponds with the flue 8, and the twyer 11<sup>a</sup> corresponds with the twyer 11.

In the furnace illustrated, the diameter of the furnace is 20 feet, and the height of the furnace above the outlet ports 7<sup>a</sup> is in the 35 neighborhood of 10 feet. Such a furnace is adapted for operation with natural draft.

The foregoing detailed description has been given for clearness of understanding only, and no unnecessary limitation should 40 be understood therefrom, but the appended claims should be construed as broadly as permissible in view of the prior art.

What I regard as new and desire to secure by Letters Patent is—

45 1. In an ore-reducing furnace, the combination with a base-portion provided with means for discharging ore and solid fuel, an upper portion provided with means for charging ore and fuel thereinto, means for supplying air to the upper portion of the furnace, and an outlet gas flue communicating with the middle portion of the furnace.

50 2. In an ore-reducing furnace, the combination of a de-oxidizing-chamber provided at its upper portion with means for introducing ore and fuel thereinto, a pre-heater having its lower portion adapted to deliver pre-heated ore and fuel to the de-oxidizing-chamber, air-admission means communicat- 55 ing with the upper portion of the de-oxidizing-chamber, and a gas flue connected with the median portion of the de-oxidizing-chamber and communicating with the lower portion of the pre-heater.

60 3. In an ore-reducing furnace, the combina-

tion of a de-oxidizing-chamber provided at its upper portion with means for introducing ore and fuel thereinto, a pre-heater having its lower portion adapted to deliver pre-heated ore and fuel to the de-oxidizing- 70 chamber, air-admission means communicating with the upper portion of the de-oxidizing-chamber, an outlet-gas flue leading from the de-oxidizing chamber some distance below the air-admission means and communicating with the lower portion of the pre-heater, and means for supplying air to the lower portion of the preheater. 75

4. In an ore-reducing furnace, the combination of a de-oxidizing-chamber having an 80 enlarged central portion and a gas flue leading therefrom, a pre-heating tube having its lower end disposed above said de-oxidizing-chamber, a closure interposed between the pre-heating tube and the de-oxidizing chamber, means for supplying air to the upper portion of the de-oxidizing-chamber, said 85 gas flue serving to discharge gas into the lower end of the pre-heating tube, means for admitting air to the lower end of the 90 pre-heating tube, and a smoke-stack connected with the upper end of the pre-heating tube.

5. In an ore-reducing furnace, the combination of a down-draft de-oxidizing-chamber, an inclined heating-tube adapted to deliver pre-heated ore and fuel to the upper portion of said chamber, means for supplying air to the upper portion of said chamber, a gas flue communicating with said 95 chamber near its median portion and serving to conduct gas to the lower portion of the pre-heating tube, and means for admitting air to the lower portion of the pre-heating tube. 100

6. In an ore-reducing furnace, the combination of a down-draft de-oxidizing-chamber, an inclined preheating-tube adapted to deliver pre-heated ore and fuel to the upper portion of said chamber, means for supplying air to the upper portion of said chamber, a gas flue communicating with said chamber near its median portion and serving to conduct gas to the lower portion of the pre-heating tube, a closure interposed between 110 the pre-heating tube and said chamber, and means connected with the upper portion of the pre-heating chamber through which fresh fuel may be charged. 115

7. In an ore-reducing furnace, the combination of a down-draft de-oxidizing-chamber having a relatively large central portion, a gas flue leading from said central portion, an inclined pre-heating tube having its lower end adapted to deliver pre-heated ore 120 and fuel to the upper portion of said chamber, said flue serving to deliver gaseous fuel to the lower portion of said pre-heating tube, and means for supplying air to the upper portion of said de-oxidizing-chamber. 125 130

8. In an ore-reducing furnace, the combination of a down-draft de-oxidizing-chamber having a relatively large central portion, a gas flue leading from said central portion, an inclined pre-heating tube having its lower end adapted to deliver pre-heated ore and fuel to the upper portion of said chamber, said flue serving to deliver gaseous fuel to the lower portion of said pre-heating tube, and means connected with the upper portion of the de-oxidizing-chamber through which fresh solid fuel may be charged. 5
9. In an ore-reducing furnace, the combination of a pre-heating tube, an elbow communicating with the lower portion thereof, a down-draft de-oxidizing-chamber beneath said elbow provided with a gas flue which extends through said elbow and serves to deliver gaseous fuel to said pre-heating tube, a closure interposed between said elbow and said de-oxidizing-chamber, and air-admission means connected with the upper portion of the de-oxidizing-chamber. 10
10. In an ore-reducing furnace, the combination of an inclined pre-heating tube, an elbow communicating with the lower portion thereof, a down-draft de-oxidizing-chamber beneath said elbow provided with a gas flue which extends through said elbow and serves to deliver gaseous fuel to said pre-heating tube, a closure interposed between said elbow and said de-oxidizing-chamber, air-admission means connected with the upper portion of the de-oxidizing-chamber. 15
11. In an ore-reducing furnace, the combination of a down-draft de-oxidizing-chamber of relatively large horizontal circumference at its median portion and relatively small height above said median portion, a gas flue communicating with the median portion of said de-oxidizing-chamber, an inclined pre-heating tube having its lower portion disposed to deliver pre-heated ore and fuel to the upper portion of the de-oxidizing-chamber, and means for regulating the admission of air to the upper portion of the de-oxidizing-chamber. 20
12. In an ore-reducing furnace, the combination of a down-draft de-oxidizing-chamber having a contracted upper end, an enlarged median portion, and a reduced lower portion, said chamber formed with a bustle-pipe at its median portion, a gas flue leading from said bustle-pipe, an inclined pre-heating tube adapted to deliver pre-heated ore and fuel to the upper portion of said chamber, and with the lower end of which said gas-flue communicates, an elbow connecting the lower portion of the pre-heating tube with the upper portion of said chamber. 25
13. In an ore-reducing furnace, the combination of a relatively low, large-area de-oxidizing-chamber equipped at its upper portion with air-admission means, a relatively long inclined pre-heating tube having its lower end disposed to deliver pre-heated ore and fuel to said chamber, and a gas-flue connecting said chambers below said air-admission means with the lower portion of said pre-heating tube. 30
14. In an ore-reducing furnace, the combination of a relatively low, large-area de-oxidizing-chamber equipped at its upper portion with air-admission means, a relatively long inclined pre-heating tube having its lower end disposed to deliver pre-heated ore and fuel to said chamber, a gas-flue connecting said chamber with the lower portion of said pre-heating tube, an elbow connecting the lower end of said pre-heating tube with the upper portion of said chamber, and a closure for the upper portion of said chamber. 35
15. In an ore-reducing furnace, the combination of a relatively low, large-area de-oxidizing-chamber equipped at its upper portion with air-admission means, a relatively long inclined pre-heating tube having its lower end disposed to deliver pre-heated ore and fuel to said chamber, a gas-flue connecting said chamber with the lower portion of said pre-heating tube, an elbow connecting the lower end of said pre-heating tube with the upper portion of said chamber, a closure for the upper portion of said chamber, and means connected with the upper portion of said chamber for enabling fresh solid fuel to be introduced into the chamber. 40
16. In an ore-reducing furnace, the combination of a relatively large pre-heating device through which ore and solid fuel may be fed slowly, a relatively low upright de-oxidizing chamber having its upper portion communicating with said pre-heating device, means for supplying air to the ore and fuel body in the de-oxidizing-chamber, and means for supplying air to the pre-heating device to burn the combustible gases passing thereto from the de-oxidizing-chamber. 45
17. In an ore-reducing furnace, the combination of a pre-heating device of relatively large dimensions, an upright de-oxidizing chamber of relatively small height and large area, said de-oxidizing chamber having communication at its upper portion with said pre-heating device, means for supplying air to the interior of the ore and fuel body. 50

within said de-oxidizing-chamber, and means for supplying air to said pre-heating device in such quantity as to consume the combustible gases therein without attacking the solid fuel.

18. In an ore-reducing furnace, the combination of a relatively large-dimensioned, inclined pre-heating tube through which ore and solid fuel may be fed slowly, a de-oxidizing-chamber communicating with the lower end of said pre-heating tube, means for supplying air to the lower portion of said pre-heating tube in such quantity as to burn the combustible gases therein without attacking the solid fuel, and natural-draft means for supplying air within the ore and fuel body in said de-oxidizing-chamber in sufficient quantity to maintain a hot de-oxidizing and metal-fusing and globing temperature in said de-oxidizing-chamber.

19. In an ore-reducing furnace, the combination of a relatively large-dimensioned, inclined pre-heating tube through which ore and solid fuel may be fed slowly, a de-oxidizing-chamber communicating with the lower end of said pre-heating tube, natural draft means for supplying air to the lower portion of said pre-heating tube in such quantity as to burn the combustible gases therein without attacking the solid fuel, natural-draft means for supplying air within the air and fuel body in said de-oxidizing-chamber in sufficient quantity to maintain a hot de-oxidizing and metal-fusing and globing temperature in said de-oxidizing-chamber, and a smoke-stack communicating with the upper end of said pre-heating tube.

20. In an ore-reducing furnace, the combination of a relatively large-dimensioned inclined pre-heating tube through which ore and solid fuel may be fed slowly, a smoke-stack communicating with the upper end thereof, a charging-device having a chute extending through said stack and adapted to deliver ore and fuel to said pre-heating tube, a relatively-low de-oxidizing-chamber having a passage communicating with the lower end of the pre-heating tube through

which combustible gases may pass, and tuyers adapted to deliver air within the fuel and ore body in said de-oxidizing-chamber in sufficient quantities to maintain a high de-oxidizing and metal-fusing temperature therein.

21. In an ore-reducing furnace, the combination of a de-oxidizing chamber adapted to support a low stack of mixed ore and fuel, means for introducing an air supply into said stack in such quantity as to provide by 60 the re-actions a metal-fusing and globing temperature in one zone and a de-oxidizing medium in another zone, a pre-heating device adapted to supply pre-heated ore and fuel to said de-oxidizing chamber to replenish said stack, said pre-heating device receiving the gases from said de-oxidizing chamber after they have served the de-oxidizing function, means for charging fresh fuel into said de-oxidizing chamber, means 70 for supplying air to said pre-heating device to burn the gases therein, and means for removing unburned fuel, gangue and metal in solid form from the bottom of the de-oxidizing chamber.

22. In an ore-reducing furnace, the combination of a de-oxidizing chamber adapted to support a low stack of mixed ore and fuel, means for introducing an air supply into said stack in such quantity as to provide by 80 the re-actions a metal-fusing and globing temperature in one zone and a de-oxidizing medium in another zone, a pre-heating device adapted to supply pre-heated ore and fuel to said de-oxidizing chamber to replenish said stack, said pre-heating device receiving the gases from said de-oxidizing chamber after they have served the de-oxidizing function, means for supplying air to 85 said pre-heating device to burn the gases therein, and means for removing unburned fuel, gangue and metal in solid form from the bottom of the de-oxidizing chamber.

ALBERT G. JONES.

In presence of—  
NELLIE B. DEARBORN,  
E. D. STEELE.